

# UNITED STATES PATENT OFFICE.

TRUMAN A. HOUSER, OF DORRANCETON, PENNSYLVANIA.

## COMPOSITION FOR TEMPERING STEEL.

1,056,277.

No Drawing.

Specification of Letters Patent. Patented Mar. 18, 1913.

Application filed November 23, 1912. Serial No. 733,221.

To all whom it may concern:

Be it known that I, TRUMAN A. HOUSER, a citizen of the United States, residing at Dorranceton, in the county of Luzerne and State of Pennsylvania, have invented certain new and useful Improvements in Compositions for Tempering Steel, of which the following is a specification.

My invention relates to the method of tempering steel and the composition of matter used in said method and has for its principal object the provision of a method by which steel may be made harder and tougher at a lower heat than by the methods now in use and furthermore, to provide means by which the tempered steel will not check or crack and will not scale after being treated.

In the practice of my invention, I employ a composition of matter comprising the following ingredients in the proportions named, viz: cyanid of potassium 4 ounces, sal-ammoniac 3 ounces, borax 3 ounces, saltpeter 2 ounces, sal-soda 2 ounces, blue vitriol 2 ounces, table salt 1 ounce, and rosin  $\frac{1}{2}$  ounce. These ingredients are powdered and thoroughly mixed while in their powdered state.

In the practice of my method in treating carbon or tool steel I first heat the steel to a dark cherry red. I then apply the compound hereabove described to the heated steel by sprinkling it thereon and return the steel to the fire until the compound flows freely over the steel. After this I dip the steel in water and draw the temper. I then try the temper with a file and repeat the above operation until the temper is satisfactory. After the proper temper has been reached I cool the steel in water.

To harden taps, reamers, dies and the like, I apply the composition above described after heating the tool to a cherry red. The tool is then returned to the fire and heated until it is a dark cherry red. I then draw a temper to the toughness desired, and cool in water.

It will be noted that one of the principal

advantages of this method is that carbon steel can be tempered at a lower heat and made harder and tougher than by any other method, and furthermore, that steel treated with this composition will not scale.

In using my improved composition for the treatment of alloy or high speed steel, I first heat the part of the tool to be tempered to a high red heat. I then cover the tool with the composition and reheat the tool to as high a heat as possible without causing it to melt. The tool is then removed from the fire and brushed off and I then place it in a bath of fish oil keeping the tool in motion in the oil to prevent the oil from becoming heated immediately surrounding the tool. In place of oil if desired, the temper may be secured by submitting the tool to a strong blast of cooled air.

By this method of treating high speed or alloy steel, it is apparent that a lower heat than by the method in present use may be employed and at the same time the steel will be harder and tougher and furthermore, the steel will not check or crack and will not scale.

Having thus described my invention what I claim is:—

1. A composition of matter for tempering steel, consisting of a certain quantity of cyanid of potassium and smaller quantities of borax, saltpeter, sal-soda, blue vitriol, table salt, and rosin.

2. A composition of matter for tempering steel consisting of cyanid of potassium 4 ounces, sal-ammoniac 3 ounces, borax 3 ounces, saltpeter 2 ounces, sal-soda 2 ounces, blue vitriol 2 ounces, table salt 1 ounce, and rosin  $\frac{1}{2}$  ounce.

In testimony whereof I affix my signature in presence of two witnesses.

TRUMAN A. HOUSER.

Witnesses:

BESS H. LLOYD,

Wm. J. RUFF.